

March 25, 1969

E. M. PROSEN

3,434,526

METHOD OF MAKING CAST MOVABLE JOINT

Original Filed Sept. 6, 1960

2+

FIG. 1.



FIG. 2.



3+

FIG. 3.



FIG. 4.



INVENTOR  
EMIL M. PROSEN

BY

Burly, Townsend, Watson & Churchill  
ATTORNEYS.

1

3,434,526

**METHOD OF MAKING CAST MOVABLE JOINT**  
 Emil M. Prosen, Bala-Cynwyd, Pa., assignor to Nobilium  
 Products, Inc., Philadelphia, Pa., a corporation of  
 Pennsylvania

Continuation of application Ser. No. 54,229, Sept. 6,  
 1960. This application Mar. 15, 1965, Ser. No. 444,900  
 Int. Cl. B22d 31/00, 23/06; B22c 9/12  
 U.S. Cl. 164—69

3 Claims

This application is a continuation of my pending application, Ser. No. 54,229, filed Sept. 6, 1960 (now abandoned) and relates to cast articulated assemblies or movable joints for use in prosthetic dentistry, and to the method of making the same.

In accordance with current practice in prosthetic dentistry where clasps on a dental restoration are provided for engagement over natural teeth to hold the restoration in place in the mouth of a wearer, the clasps are rigidly held by the restoration and are immovably held on the natural teeth and as a concomitant thereof the clasps must move with movement of the restoration during mastication. Such movement imposes a severe strain on the teeth over which the clasps are applied and causes frequently, not only discomfort to the wearer of the restoration but also loosening of the clasped teeth. Although numerous attempts have been made to remedy the aforementioned shortcoming in mounting clasps of dental restorations, so far as I am aware none of the structures proposed and applied to noble metals and high melting point alloys used in dental restorations have proven satisfactory.

Accordingly, it is an object of the present invention to provide a cast articulated assembly or movable joint for use in prosthetic dentistry, wherein limited movement in all directions is provided between the parts at the joint.

A more specific object of the invention is to provide a dental restoration comprising a cast metal support with tooth clasps, which restoration is capable of independent limited movement or play in all directions relative to the clasps.

A further object of the invention is to provide a novel method of procedure in forming tooth clasps on cast metal dental restorations whereby the metal support for the clasps will be capable of limited movement in all directions in relation to the clasps.

The foregoing and other objects of the invention, not specifically enumerated, I accomplish by forming one of the members of the cast movable joint with a projection which is to be engaged within a socket in the other member of the cast metal joint, then applying to the projection a coating composition to a thickness corresponding to the amount of freedom of movement desired in the joint between the members; then applying said coated cast member on a refractory model after which said model and said first mentioned member are fully waxed and invested and the wax then melted out to provide a mould within which a casting is made in the usual manner. Such casting consisting of both members in firm engagement is then removed from the mould. The casting is then treated to dissolve away the coating composition, thus leaving the first and second members of the joint in assembled relation with the desired freedom of movement or play therebetween. The invention will be better understood from the detailed description which follows when considered in connection with the accompanying drawing wherein:

FIG. 1 is a top plan view of a dental restoration embodying the invention, shown in relation to natural teeth over which the restoration is to be removably anchored, the restored teeth being omitted from the restoration.

FIG. 2 is a section taken along the line 2—2 of FIG. 1.

2

FIG. 3 is a section taken along the line 3—3 of FIG. 2.

FIG. 4 is a section of a preformed clasp member having a soluble heat refractory coating applied to a portion thereof prior to having the supporting part of the restoration cast around the coated portion of the clasp.

In the drawing wherein I have shown my invention applied to a dental restoration for the lower jaw of a human mouth, the reference character 10 indicates natural teeth, shown in phantom, in relation to which a dental restoration 11 is applied. The restoration, which is merely illustrative consists of a pair of saddle members 12 having artificial teeth (not shown) mounted thereon, the saddles being supportable on the lower alveolar ridge and joined together by a lingual connecting bar 13, each saddle having floatingly mounted therein a tooth clasp 14 having a plurality of prongs 14a, 14b and 14c engageable over a second premolar to hold the restoration in place.

According to the present invention the clasps on the saddles are such as to provide for limited relative movement or play in all direction of the saddles relative to the clasps so that during mastication the slight movements of the saddles will not be transmitted to the clasps and as a concomitant thereof impose stresses on the teeth upon which the clasps are anchored. To this end provision is made for limited spatial movement or play in all directions for the saddles relative to the clasps. This is accomplished by forming the clasps and saddles with interengaged substantially complementary non-removable parts 16 and sockets 17 respectively, part 16 being a hook-shaped projection on the clasp similar in form and of somewhat smaller size in all dimensions than the socket 17 in the saddle.

To provide the desired freedom of movement of the saddles relatively to the clasps, each clasp 14 consisting of the prongs 14a, 14b, 14c and the hook-shaped projection 16 is preformed in wax on a refractory model of the toothed jaw, and is then cast by the well-known lost wax procedure. The hook-shaped projections 16 of the cast clasps are then coated with a chemically soluble high heat-resistant refractory substance 18 to a thickness corresponding to the extent of movement desired between the saddles and the clasps. The coating may be either a frit-like coating substance or a metal deposit formed by electro-plating. A suitable frit-like coating substance has the following composition: water 810 cc., sodium silicate 945 cc., wetting agent 2.5 cc., silica flour 1300 gr., zirconium silicate 2300 gr., chromic oxide 20 gr. The frit-like composition may be painted onto or otherwise applied to the projections and caused to set thereon by being subjected to a temperature of approximately 1400° F. Where the coating is a metal applied by electro-plating, it is preferable that said metal be nickel which can be dissolved away by an acid which will not attack the noble metals or the non-precious metal alloys used in making dental restorations.

The clasps as thus coated are placed on a refractory model which is a reproduction of the original model and the model is then fully waxed to provide for the entire metal casting required for the saddles 12, the connecting bar 13, and the coated projections 16 of the clasps. The waxed-up model is then invested with a refractory case and the wax then melted out to provide a mould space in which the casting is made in the usual manner. The casting which is in firm engagement with the projections on the preformed clasps is then removed from the case, cleaned of the refractory material and the sprues cut away.

To remove the heat refractory frit-like coating from the clasp projections which are embedded in the composite casting, said casting is treated in boiling sodium hydroxide for about 30 minutes to dissolve the coating,

thus providing the limited space or socket within the saddles to permit relative movement between said saddles and clasps. As some sodium hydroxide may remain and solidify at room temperature within the space thus provided between the projections on the clasps and saddles such remaining sodium hydroxide may be removed by treating the casting in a 50% nitric acid solution and the casting then rinsed with water.

If nickel plating is employed to provide the heat refractory coating on the projections of the clasps, such coating can be removed by treating the casting in hot nitric acid until all of the deposited nickel is dissolved away to provide the sockets within the saddles around the projections on the clasps.

After the clasps are mounted in the saddles to provide the freedom of movement between said parts, the dental restoration may be finished in a manner well understood by a dental mechanic.

Although I have shown and described a preferred embodiment of my invention as applied to a dental restoration having two saddles, two clasps and a connecting bar between the saddles, it will be understood that the technique described could be employed in breaking the rigidity in the structure of a dental appliance, for example intermediate or at the ends of a connecting bar. Accordingly, the foregoing description and drawing are to be considered as exemplary and not in a limiting sense and is to be construed within the scope of the appended claims.

What I claim is:

1. The method of forming a removable dental restoration having a tooth clasp and a supporting part for the clasp, in which restoration the supporting part has a socket therein and the clasp has a projection of a shape similar to, smaller than and engaged non-removably in said socket so as to provide for limited free play movement of the supporting part in all directions relative to said projection, said method comprising first preforming a casting by the lost wax technique of the clasp and its projection from a wax-up of the clasp and its projection on a refractory model, coating the projection on the clasp with a chemically soluble high heat-resistant refractory substance to a thickness corresponding to the extent of movement desired for the supporting part relatively to the clasp, firing said refractory substance, mounting the cast coated clasp on the aforementioned refractory model, forming a wax-up of the supporting part around the coated projection investing the resulting model, melting out the wax to provide a mould, casting the supporting part around the coated projection on the clasp, removing the casting from the mould and dissolving away the

refractory coating substance to provide a pocket clearance in said casting corresponding to the thickness of said heat-resistant refractory coating.

2. The method according to claim 1 wherein the coating substance is a frit-like composition which after firing is soluble in boiling alkali.

3. The method of forming a removable dental restoration having a tooth clasp and a supporting part for the clasp, in which restoration the supporting part has a socket therein and the clasp has a projection of a shape similar to, smaller than and engaged non-removably in said socket so as to provide for limited free play movement of the supporting part in all directions relative to said projection, said method comprising first preforming a casting by the lost wax technique of the clasp and its projection from a wax-up of the clasp and its projection on a refractory model, coating the projection on the clasp with a chemically soluble high heat-resistant refractory substance to a thickness corresponding to the extent of movement desired for the supporting part relatively to the clasp, mounting the cast coated clasp on the aforementioned refractory model, forming a wax-up of the supporting part around the casted projection investing the resulting model, melting out the wax to provide a mould, casting the supporting part around the coated projection on the clasp, removing the casting from the mould and dissolving away the refractory coating substance to provide a pocket clearance in said casting corresponding to the thickness of said heat-resistant refractory coating, and wherein the coating substance is a metal plating which is soluble in a reagent which is non-reactive to the metals forming the clasp and the supporting member.

#### References Cited

#### UNITED STATES PATENTS

|           |        |                        |
|-----------|--------|------------------------|
| 2,546,397 | 3/1951 | Johnson.               |
| 2,550,436 | 4/1951 | Yates ----- 32-7       |
| 1,657,476 | 1/1928 | Inami ----- 22-190.1   |
| 2,042,330 | 5/1936 | Bradley ----- 22-190.1 |
| 2,196,505 | 4/1940 | Morton ----- 32-6      |
| 2,227,735 | 1/1941 | Morton ----- 32-6      |
| 2,797,482 | 7/1957 | Zahn ----- 32-5        |
| 2,628,166 | 2/1953 | Haller ----- 164-90 X  |

45 J. SPENCER OVERHOLSER, Primary Examiner.

V. K. RISING, Assistant Examiner.

U.S. CL. X.R.

32-7; 164-12, 90, 36, 111; 249-54, 98, 61; 106-38.3